# EUROPEAN PATENT SPECIFICATION

(11) **EP 3 908 413 B1**
(45) Date of publication and mention of the grant of the patent: **30.10.2024**
(21) Application number: 19948143.3
(22) Date of filing: 30.09.2019
(51) Int. Cl.: B41M 5/52, B41M 5/50, B05D 5/00, B05D 5/04, B05D 1/26, B05D 7/00

(54) **PRINTABLE RECORDING MEDIA**
BEDRUCKBARES AUFZEICHNUNGSMEDIUM
SUPPORT D'ENREGISTREMENT IMPRIMABLE

(43) Date of publication of application: 17.11.2021
(73) Proprietor: Hewlett-Packard Development Company, L.P., Spring TX 77389 (US)
(72) Inventor: ZHOU, Xiaoqi, San Diego, California 92127-1899 (US); BRANDSTEIN, Or, San Diego, California 92127-1899 (US); FU, Xulong, San Diego, California 92127-1899 (US)
(74) Representative: Plasseraud IP
(86) International application number: PCT/US2019/053755
(87) International publication number: WO 2021/066787

(56) References cited:
- US-A1- 2002 142 139
- US-A1- 2002 142 140
- US-A1- 2003 087 112
- US-A1- 2004 109 958
- US-A1- 2004 152 027
- US-A1- 2005 065 235
- US-A1- 2009 035 478
- US-A1- 2014 202 749

## Description

### BACKGROUND

Inkjet printing is a non-impact printing method in which an electronic signal controls and directs droplets or a stream of ink that can be deposited on a variety of substrates. Current inkjet printing technology involves forcing the ink drops through small nozzles by thermal ejection, piezoelectric pressure or oscillation, onto the surface of a media. This technology has become a popular way of recording images on various media surfaces, particularly paper, for many reasons, including low printer noise, capability of high-speed recording and multi-color recording. Inkjet web printing is a technology that is specifically well adapted for commercial and industrial printing. It has rapidly become apparent that the image quality of printed images using such printing technology is strongly dependent on the construction of the recording media used. Consequently, improved recording media, often specifically designed, have been developed. US2004/109958A1 describes a highly reflective and light-emitting printable recording medium comprising two layers coated on a paper. US2014/202749A1 is concerned with printing a conductive pattern on a media which contains melamine as crosslinker. US2002/142140A1 and US2002/142139A1 describe a single layer coating on a recording medium comprising as crosslinkers for example carbodiimides or epoxides.

### BRIEF DESCRIPTION OF THE DRAWING

The drawings illustrate various examples of the present printable recording media and are part of the specification. Figure 1, Figure 2, Figure 3 and Figure 4 are a cross-sectional view of the printable recording media according to some examples of the present disclosure. Figure 5 is a flowchart illustrating a method for producing the printable recording media according to one example of the present disclosure.

### DETAILED DESCRIPTION

When using inkjet printing technology challenges exist due to the specific nature of substrate, i.e. the printable recording media, that would receive the ink and therefore creating the printed image. It is highly desirable for the customer to have a gloss, excellent printing image quality and image durability against any mechanical actions. This kind of quality is often achieved through the use of coated paper but the coating often brings the challenge to fast drying and high image durability. Due to the concern of jettability of printing head (long time printing, high volume jetting and elevated temperature), it is ideal to keep minimal amount of binder in printing ink but this has seriously bring the impact to the durability of printing image under a mechanical force like scratch or rubbing. Accordingly, investigations continue into developing printable recording media that can be effectively used with such technology and which impart good printing performances. As one example, this invention disclosed a coated media which has those characteristics. The coated media is referred to as printable recording media or printable medium.

The present disclosure is drawn to a printable recording media as defined in the appended set of claims, or printable medium, with an image-side and a back-side, comprising a base substrate with an image-side and a back-side and an ink-receiving layer, applied to the image-side of the base substrate, comprising a reactive crosslinking agent, inorganic pigment particles or a mixture of inorganic particles, and polymeric binders or a mixture of polymeric binders. The printable medium further comprises a primary layer containing, at least, inorganic pigment particles or a mixture of inorganic particles and polymeric binders or a mixture of polymeric binders, that is applied on the image-side of the base substrate, below the ink-receiving layer.

The present disclosure also relates to a method for forming said printable recording media and to the printing method using said printable medium. The method for forming a printable recording media comprises providing a base substrate, with an image-side and a backside; applying an ink-receiving layer comprising a reactive crosslinking agent, inorganic pigment particles or a mixture of inorganic particles, and polymeric binders or a mixture of polymeric binders to the image-side of the base substrate and drying the coating composition to remove water from the media substrate to leave an ink-receiving layer thereon.

The printable recording media, or printable medium, according to the present disclosure is particularly well suited for inkjet printing technology and application. In some examples, the printable media is well adapted to be used in web press applications with high speed print rates, e.g., using the HP T200 Web Press or HP T300 Web Press at rates of 304.8 meter/minute (1000 feet per minute) or more. In some other examples, printable media is to be printed with inkjet printing technology such as "HP Page Wide Array printing" where more than hundreds of thousand tiny nozzles on a stationary print-head that spans the width of a page, delivering multicolors ink onto a moving sheet of paper under a single pass to achieve the super-fast printing speed. Printing applications which benefit from high grade printing media, such as magazines, catalogs, books, manuals, direct mails, labels, or other similar print jobs, where large volumes of high-quality glossy image is printed very quickly, are particularly advantaged by the printable recording media described herein.

The media, according to the present disclosure, is a coated printable recording media. By "coated", it is meant herein that the printable recording media has been applied a composition. It is noted that the term "coating composition" refers to either a composition used to form a coating layer as well as the coating layer itself, the context dictating which is applicable. For example, a coating composition or coating that includes an evaporable solvent is referring to the compositional coating that is applied to a media substrate. Once coated on a media substrate and after the evaporable solvent is removed, the resulting coating layer can also be referred to as a coating. The coating composition can be applied to various media to improve, for example, printing characteristics and attributes of an image. In some examples, the coating composition is a composition that is going to be applied to an uncoated printable recording media. By "uncoated", it is meant herein that the printable recording media has not been treated or coated by any composition.

The coated media, according to the present disclosure, is a printable recording medium (or printable media) that provide printed images that have outstanding print durability and excellent scratch resistance while maintaining good printing characteristics and image quality (i.e. printing performance). As good printing characteristics, it is meant herein good black optical density, good color gamut and sharpness of the printed image. The images printed on the printable recording media will thus be able to impart excellent image quality: vivid color, such as higher gamut and high color density. High print density and color gamut volume are realized with substantially no visual color-to-color bleed and with good coalescence characteristics.

The images printed on the printable recording media will also have excellent durability and excellent scratch resistance; specifically, it will have excellent durability under mechanical actions such as rubbing and scratching. By "scratch resistance", it is meant herein that the composition is resistant to any modes of scratching which include, scuff and abrasion. By the term "scuff', it is meant herein damages to a print due to dragging something blunt across it (like brushing fingertips along printed image). Scuffs do not usually remove colorant, but they do tend to change the gloss of the area that was scuffed. By the term "abrasion", it is meant herein the damage to a print due to wearing, grinding or rubbing away due to friction. Abrasion is correlated with removal of colorant (i.e. with the OD loss).

Figure 1, Figure 2, Figure 3 and Figure 4 schematically illustrate some examples of the printable recording media (100) as described herein. Figure 5 is a flowchart illustrating an example of a method for producing the printable recording media. As will be appreciated by those skilled in the art, Figure 1, Figure 2, Figure 3 and Figure 4 illustrate the relative positioning of the various layers of the printable media without necessarily illustrating the relative thicknesses of the various layers. It is to be understood that the thickness of the various layers is exaggerated for illustrative purposes.

Figure 1 illustrates the printable recording media (100) as described herein. The printable recording media (100) encompasses a base substrate or media substrate or bottom supporting substrate (110) and an ink-receiving layer (120). The ink-receiving layer is applied on, at least, one side of the substrate (110) in order to from an image-receiving layer (120). The ink-receiving layer composition is thus applied on one side, i.e. the image side, only and no other coating is applied on opposite side. The image side with the image-receiving layer is considered as the side where the image will be printed. The printable media (100) has two surfaces: a first surface which might be referred to as the "image-receiving side", "image surface" or "image side" (101) when coated with the image-receiving layer and the primary layer, and a second surface, the opposite surface, which might be referred to as the "back surface" or "back-side" (102).

Figure 2 illustrates another example of the printable recording media (100) as described herein. The printable media (100) encompasses a base substrate (110) with image-receiving coating layers (120) that are applied to both the "image side" (101) and the "back-side" (102) of the print media. In theory, both the image side and the back-side could be printed and functionalized as image-receiving layer.

Figure 3 illustrates another example of the printable recording media (100) as described herein. The printable recording media (100) encompasses a base substrate (110), a primary layer (130) applied on, at least, one side of the base substrate, over the base substrate (110) and below the image-receiving coating layer (120). In some examples, such as illustrated in Figure 3, the printable media (100) encompasses thus a base substrate (110), a primary layer (130) and an image-receiving coating layer (120) applied only on the image-side (101) of the printable recording media (100). In yet some other examples, such as illustrated in Figure 4, the printable media (100) encompasses a base substrate (110) with primary layers (130) that are applied on both sides, on the image (101) and on the back-side (102), of the base substrate (110). Image-receiving coating layers (120) are applied over both primary layer (130) on both sides of the printable recording media (100). In theory, both the image side and the back-side could thus be printed.

An example of a method (200) for forming a printable recording media in accordance with the principles described herein, by way of illustration and not limitation, is shown in Figure 5. As illustrated in Figure 5, such method encompasses providing (210) a base substrate, with an image-side and a back-side, applying (210) an ink-receiving layer comprising a reactive crosslinking agent, inorganic pigment particles or a mixture of inorganic particles, and polymeric binders or a mixture of polymeric binders to the image-side of the base substrate and drying (220) the coating composition to remove water from the media substrate to leave an ink-receiving layer thereon in order to obtain the printable recording media.

The present disclosure relates thus also to a coated printable recording media, with an image-side (101) and a back-side (102), comprising a base substrate (110) and an image-receiving layer (120), that comprises, at least, a reactive crosslinking agent, inorganic pigment particles or a mixture of inorganic particles, and polymeric binder or a mixture of polymeric binders. Such layer is called "image-receiving layer" since, during the printing process, the ink will be directly deposited on its surface. In some other examples, the printable recording media comprises a base substrate (110) and ink-receiving layers (120), comprising a reactive crosslinking agent, inorganic pigment particles or a mixture of inorganic particles, and polymeric binder or a mixture of polymeric binders, that are applied to both opposing sides of the base substrate
In some examples, the ink-receiving layer can further comprise, as optional ingredients, fixative agents. In some other examples, the ink-receiving layer can further comprise, as optional ingredients, COF (coefficient of friction) controlling agents. In yet some other examples, the ink-receiving layer might further comprise, as optional ingredients, ink colorant fixing agents, surfactant and/or other processing aids such as pH control agent, deformer and biocide.

The ink-receiving layer (120) can be disposed on the image-side (101) of the base substrate (110), at a coat-weight in the range of about 0.1 to about 40 gram per square meter (g/m2 or gsm), or in the range of about 1 gsm to about 20 gsm, or in the range of about 3 to about 15 gsm. In some other examples, ink-receiving layers (120) are disposed on the image-side (101) and on the back-side (102) of the base substrate (110), at a coat-weight in the range of about 0.1 to about 40 gram per square meter (g/m2 or gsm), or in the range of about 1 gsm to about 20 gsm, or in the range of about 3 to about 15 gsm.

The printable recording media (100) comprises a base substrate (110); a primary layer (130) and an image-receiving coating layer (120) wherein the primary layer (130) is applied directly on, at least, one side of the base substrate (i.e. the image side), below the image-receiving coating composition. In some other examples, the primary layer is applied on both the image-side and the back-side of the media base substrate. The primary layer comprises, at least, inorganic pigment particles or a mixture of inorganic particles and polymeric binder or a mixture of polymeric binders. The primary layer might further comprises optional ingredients, such as ink colorant fixing agents, surfactant and/or other processing aids such as pH control agent, deformer and biocide.

The primary layer (130) can be disposed on the image-side (101) of the base substrate (110), below the image-receiving coating layer (120), at a coat-weight in the range of about 3 to about 50 gram per square meter (g/m2 or gsm), or in the range of about 5 gsm to about 10 gsm. In some other examples, primary layers (130) are disposed on the image-side (101) and on the back-side (102) of the base substrate (110), below the image-receiving coating layer (120), at a coat-weight in the range of about 3 to about 50 gram per square meter (g/m2 or gsm), or in the range of about 5 gsm to about 10 gsm.

The components of both the image-receiving coating layer (120) and of the primary layer (130), i.e. the inorganic pigment particles or the mixture of inorganic particles, the polymeric binder or the mixture of polymeric binders and also the other optional ingredients, surfactants and other processing aids for examples, can be the same in one example, or can be different in another example. The details of each composition component are described below.

The printable recording media comprises, at least, an ink-receiving layer (120) composition that includes a reactive crosslinking agent. The reactive crosslinking agent can be defined as a chemical with functional groups that is capable of forming a crosslinking reaction with other reactive groups such as amine, carboxyl, hydroxyl, and thiol, of the media substrate, and of the binders present in the pigmented inks, for examples, upon certain condition such as heating at 50°C to 200°C for examples.

The reactive crosslinking agent can have a weight average molecular weight ranging from about 100 to about 3,000,000. In some examples, the weight average molecular weight of the reactive crosslinking agent ranges from about 100 to about 1,000,000; or from about 200 to about 500,000; or from about 300 to about 200,000 ; or from about 300 to about 100,000. In some other examples, the reactive crosslinking agent has a weight average molecular weight of 100,000 or less. In yet some other examples, the weight average molecular weight of the reactive crosslinking agent ranges from about 500 to about 40,000. Any weight average molecular weight throughout this disclosure is in Daltons.

In an example, the reactive crosslinking agent is present in the ink-receiving layer, in an amount ranging from about 0.5 wt % active to about 15 wt % active based on a total weight of the ink-receiving layer composition. In further examples, the reactive crosslinking agent is present in an amount ranging from about 1 wt % active to about 10 wt % active; or from about 4 wt % active to about 8 wt % active; or from about 2 wt % active to about 7 wt % active; or from about 6 wt % active to about 10 wt % active, based on a total weight of the ink-receiving layer composition.

In some example, the crosslink agent is heterocyclic ammonium salt. In some other example, the heterocyclic ammonium salt is a polymeric salt consisting of four membered heterocyclic rings containing a quaternary ammonium as shown in the Formula 1 :

In Formula 1, R³ is hydroxyl group, carboxy, acetoxy, alkoxy, amino or alkyl group, for example, at the 3'-position. R¹ and R² are groups at the 1,1'-nitrogen position and connecting the group to the backbone polymeric in long chain structure that can be polyamide chain and polyalkylenepolyamine chain. The backbone polymeric structure includes, but is not limited to, polyethylene imine, polyamidoamine, the polyamidoaminester, or polyester backbone with pendant secondary amine groups.

When R³ is hydroxyl group, the structure is called azetidinium salts. Such azetidinium salts can be available from the reaction from either primary amine or secondary amine with epichlorohydrin by two-step reaction as shown in equations 1 and 2.

The polymeric heterocyclic salt can be commercially available, for example, under the tradename Beetle^{®} PT746 from BIP (Oldbury) Ltd, Polycup serial from Solenis, Inc such as Polycup^{®} 8210, Polycup^{®} 9200, Polycup^{®} 7535, Polycup^{®} 7360A, Polycup^{®} 2000, Polycup^{®} 172 and Polycup^{®} 9700.

The reactive crosslinking agent comprised in the printable recording media is an azetidinium-containing polyamine polymer. In some other examples, the reactive crosslinking agent is a polyamine epichlorohydrin resins. In yet some other examples, the reactive crosslinking agent can be selected from the group consisting of poly(diallyldimethylammonium chloride); poly(methylene-co-guanidine) anion, wherein the anion is selected from the group consisting of hydrochloride, bromide, nitrate, sulfate, and sulfonates; a polyamine; poly(dimethylamine-co-epichlorohydrin); a polyethyleneimine; a polyamide epichlorohydrin resin; a polyamine epichlorohydrin resin; and a combination thereof.

The azetidinium-containing polyamine selected for use can include any of a number of cationic polyamines with a plurality of azetidinium groups. In an un-crosslinked state, as shown in Formula 2 below, an azetidinium group generally has a structure as follows:

As shown in Formula 2, this structure is not intended to show repeating units, but rather merely a polymer that includes the azetidinium groups shown in Formula 2, including azetidinium-containing polyamines having a weight average molecular weight from 1,000 Mw to 2,000,000 Mw, from 2,000 Mw to 1,000,000 Mw, from 5,000 Mw to 200,000 Mw, from 5,000 Mw to 100,000 Mw, or from 20,000 to 1,000,000 Mw, for example. The asterisks (*) in Formula 2 represent portions of the various organic groups, polymeric portions, functional moieties, etc., for example.

In some examples, the reactive crosslinking agent including the azetidinium-containing polyamine can be derived from the reaction of a polyalkylene polyamine (e.g. ethylenediamine, bishexamethylenetriamine, and hexamethylenediamine, for example) with an epihalohydrin (e.g. epichlorohydrin, for example) (referred to as PAmE resins). In some specific examples, the reactive crosslinking agent including an azetidinium-containing polyamine can include the structure: where R₁ can be a substituted or unsubstituted C₂-C₁₂ linear alkyl group and R² is H or CH₃. In some additional examples, R₁ can be a C₂-C₁₀, C₂-C₈, or C₂-C₆ linear alkyl group. More generally, there can be from 2 to 12 carbon atoms between amine groups (including azetidinium groups) in the azetidinium-containing polyamine. In other examples, there can be from 2 to 10, from 2 to 8, or from 2 to 6 carbon atoms between amine groups in the azetidinium-containing polyamine. In some examples, where R₁ is a C₃-C₁₂ (or C₃-C₁₀, C₃-C₈, C₃-C₆, etc.) linear alkyl group, a carbon atom along the alkyl chain can be a carbonyl carbon, with the proviso that the carbonyl carbon does not form part of an amide group (i.e. R₁ does not include or form part of an amide group). In some additional examples, a carbon atom of R₁ can include a pendent hydroxyl group. The number of units as shown in Formula 3 can be any number of units that results in an azetidinium-containing polyamine having a weight average molecular weight from 1,000 Mw to 2,000,000 Mw, from 2,000 Mw to 1,000,000 Mw, from 5,000 Mw to 200,000 Mw, from 5,000 Mw to 100,000 Mw, or from 20,000 to 1,000,000 Mw, for example. These units can be repeating along the polymer, along portions of the polymer, and/or can have other moieties between individual units shown in Formula 3. Thus, the asterisks (*) in Formula 3 represent portions of polymer that are not shown, but could include various organic groups, polymeric portions, functional moieties, etc., for example.

As can be seen in Formula 3, the azetidinium-containing polyamine can include a quaternary amine (e.g. azetidinium group) and a non-quaternary amine (i.e. a primary amine, a secondary amine, a tertiary amine, or a combination thereof). In some specific examples, the azetidinium-containing polyamine can include a quaternary amine and a tertiary amine. In some additional examples, the azetidinium-containing polyamine can include a quaternary amine and a secondary amine. In some further examples, the azetidinium-containing polyamine can include a quaternary amine and a primary amine. It is noted that, in some examples, some of the azetidinium groups of the azetidinium-containing polyamine can be crosslinked to a second functional group along the azetidinium-containing polyamine. Whether or not this is the case, the azetidinium-containing polyamine can have a ratio of crosslinked or un-crosslinked azetidinium groups to other amine groups of from 0.1: 1 to 10: 1, from 0.1: 1 to 5:1, or from 1: 1 to 10:1. In other examples, the azetidinium-containing polyamine can have a ratio of crosslinked or un-crosslinked azetidinium groups to other amine groups of from 0.5: 1 to 2:1.

Non-limiting examples of commercially available azetidinium-containing polyamines that fall within these ranges of azetidinium group to amine groups include Crepetrol^{®} 73, Kymene^{®}736, Polycup^{®} 1884, Polycup^{®} 7360, and Polycup^{®} 7360A, which are available from Solenis LLC (Delaware, USA). Other compounds from this or other companies can likewise be used. With more specific detail regarding the Polycup^{®} family of azetidinium-containing polyamines, these resins tend to be formaldehyde-free, water-based crosslinking resins that are reactive with amine groups, carboxyl groups, hydroxyl groups, and thiol groups. Many of these types of groups can be present at the surface of substrates, so in addition to crosslinking that may occur with the polyurethanes that are present in the ink compositions, there can be additional crosslinking at the surface of the print media substrate. The azetidinium-containing polyamines, such as these Polycup^{®} brand resins, in conjunction with the second quaternary amine-containing polymer that is also present in the coating composition. As one specific example, Polycup^{®} 7360 is a thermosetting polyamine epichlorohydrin that can include the polymer in a fluid carrier at about 38 wt % solids and can have a range of viscosities from about 0.18 Pa•s (180 cP) to about 0.3 Pa•s (300 cP) at 25 °C, for example.

In some other examples, the reactive crosslinking agent could be a diallylazetidium salt (Formula 4), a bis(2-methoxyethyl)azetidinium salt (Formula 5), a nonylpropylazetidinium salt (Formula 6), a undecylmethylazetidinium salt (Formula 7) or a nonylpropargylazetidinium salt (Formula 8). The reactive crosslinking agent could be used a single reactive crosslinking agent or in combination with different reactive crosslinking agent.

The following Equations 3-9 are additional examples of azetidinium salts based crosslinkers that can be made from the reaction of polyetheramines (such as Jeffamine^{®}) with epichlorohydrin compounds.

The printable recording media of the present disclosure comprises an ink-receiving layer (120) containing inorganic pigment particles or a mixture of inorganic particles. The primary layer also comprises inorganic pigment particles or a mixture of inorganic particles. The inorganic pigment particles or mixture of inorganic particles can be the same or different from each other.

The ink-receiving layer (120) composition and the primary layer (130) include at least one type of pigment particles, or a mixture of different types of particulate fillers. The wording "type" refers chemical composition, crystalline structure, particle size and size distribution, and chemical and physical condition of the particle surface such as surfactant treated and high temperature calcined. In one example, the particulate filler is clay or calcium carbonate particles, such as ground calcium carbonate (GCC) or precipitated calcium carbonate (PCC). In some examples, the clay particles and calcium carbonated particles of the various types described above, can be co-dispersed in the coating layer with other particulate fillers. The dispersion of the particles or mixture of the particles is compatible with the reactive crosslinking agent, meaning thus that there is no precipitation when mixing.

Other particulate fillers that can be used in addition to the calcium carbonate particles include inorganic fillers which can generate micro-porous structure to improved ink absorbing. Examples include fumed silica and silica gels, as well as certain structured pigments. Structured pigments include those particles which have been prepared specifically to create a micro-porous structure. Examples of these structured pigments include calcine clays or porous clays that are reaction products of clay with colloidal silica. Other inorganic particles such as particles of titanium dioxide (TiO₂), silicon dioxide (SiO₂), aluminum trihydroxide (ATH), calcium carbonate (CaCOs), or zirconium oxide (ZrO₂) can be present, or these compounds can be present in forms that are inter-calcined into the structured clay. In one example, the inorganic pigment particles may be substantially non-porous mineral particles that have a special morphology that can produce a porous coating structure when solidified into a coating layer.

The ink-receiving layer (120) can include at least one type of particulate filler, or a mixture of different types particulate fillers. There is no specific limitation in selecting chemistry of particulate fillers, as long as these fillers have no chemical reactions in the solution of image receiving coating mixture before coating, where the pH of mixture is normally ranged between 4.5 to 6.5. The particulate fillers can be selected from, for example, kaolin, Kailin clays, barium sulfate, titanium dioxide, zinc oxide, zinc sulfide, satin white, aluminum silicate, diatomite, calcium silicate, magnesium silicate, synthetic amorphous silica, colloidal silica, colloidal alumina, pseudo-boehmite, aluminum hydroxide, alumina, lithopone, zeolite, and various combinations. In one example, particulate fillers are selected from the group consisting of silica, clay, kaolin, talc, titanium dioxide, and zeolites. In another example, the filler particles used are in a dry-powder form or in a form of an aqueous suspension referred as slurry with cationic charged dispersion agent since most anionic charged dispersing agent will be crashed by reactive cross-linking agent described above.

Further, in another embodiment, the inorganic pigments are porous inorganic pigments. Porous inorganic pigments refer to pigment that include a plurality of pore structures to provide a high degree of absorption capacity for liquid ink vehicle via capillary action or other similar means. Examples of porous inorganic pigments include, but are not limited to, synthesized amorphous silica, colloidal silica, alumina, colloidal alumina, and pseudo-boehmite (aluminum oxide/hydroxide). In another embodiment, the porous inorganic pigments are mixed with low surface area inorganic pigments and/or organic pigments at a weight percent ratio raging from about 5 % to about 40% of porous inorganic pigments. This mixture has the benefit of improving the ink absorption while not sacrificing other physical performance attributes such as gloss.

Precipitated calcium carbonate can be commercially available, for example, under the tradenames Opacarb^{®}A40 and Albacar^{®} (both available from Minerals Technologies Inc.). Ground calcium carbonate is commercially available, for example, under the trade names Omyafil^{®}, Hydrocarb^{®}70 and Omyapaque^{®} (all of which are available from Omya North America). Examples of commercially available filler clays are Kaocal^{®}, EG-44, and B-80 (available from Thiele Kaolin Company). An example of commercially available talc is Finntalc^{®}F03 (available from Mondo Minerals).

In some examples, inorganic pigment particles and/or mixture inorganic particles can be present, in the ink-receiving layer and/or in the primary layer composition, in an amount representing from about 50 wt % to about 92 wt % , or in an amount representing from about from about 70 wt % to about 90 wt %, or in an amount representing from about from about 80 wt % to about 88 wt % based on the total dry weight of the coating layer(s).

The printable recording media of the present disclosure comprises an ink-receiving layer (120) containing polymeric binders or a mixture of polymeric binders. The primary layer (130) also comprises polymeric binders or a mixture of polymeric binders. The polymeric binders or the mixture of polymeric binders present in the ink-receiving layer may or may not be the same from the one present in the primary layer.

In one example, the polymeric binder or the mixture of polymeric binders can be present in the ink-receiving layer and/or in the primary layer, in an amount representing from about 1 wt % to about 18 wt % with respect to the total dry weight of the coating layer. In another example, the polymeric binder or mixture of polymeric binders can be present in the ink-receiving layer and/or in the primary layer in an amount from about 3 wt % to about 13 wt % with respect to the total dry weight of the coating layer. As a further example, the polymeric binder or mixture of polymeric binders can be present in the ink-receiving layer and/or in the primary layer in an amount of from about 5 wt % to about 12 wt % with respect to the total dry weight of the coating layer(s).

The polymeric binder can be selected from synthetic and natural polymeric compounds as long as they are compatible with the reactive crosslinking agent, meaning thus that no precipitation occurs when mixing. In some examples, the polymeric binder is a water-dispersible polymeric binder or a water-soluble polymeric binder or a combination thereof. In some other examples, the polymeric binder can include both water-dispersible polymeric binder and water-soluble polymeric binder.

The ratio of water-soluble polymeric binders to water-dispersible polymeric binders can be of any value as long as such mixture provides a good adhesion to the substrate, to coating layers and to inorganic particles. In some examples, the polymeric binders can be a mixture of a water-dispersible polymeric binders and water-soluble polymeric binders that are present, in the ink-receiving layer, at a dry weight ratio of 1:25 to 1: 1, 1:20 to 3:10, or 1:20 to 4:7, for example.

Water-dispersible binders can include conjugated diene copolymer latexes, such as styrene-butadiene copolymer or acrylonitrile-butadiene copolymer; acrylic copolymer latexes, such as polymer of acrylic acid ester or methacrylic acid ester or methyl methacrylate-butadiene copolymer; vinyl copolymer latexes, such as ethylene-vinyl acetate copolymer and vinyl chloride-vinyl acetate copolymer; urethane resin latexes; alkyd resin latexes; unsaturated polyester resin latexes; and thermosetting synthetic resins, such as melamine resins and urea resins, and combinations thereof. In some examples, the water-dispersible polymer can include polymeric latex or polymeric emulsion where the polymeric core surrounded by surfactant with mid to large molecular weight polymer. The polymeric core can be dispersed by a continuous liquid phase to form an emulsion-like composition. Examples of water-dispersible polymers include, but are not limited to, acrylic polymers or copolymers latex, vinyl acetate latex, polyesters latex, vinylidene chloride latex, styrene-butadiene latex, acrylonitrile-butadiene copolymers latex, styrene acrylic copolymer latexes, and/or the like

Generally, the water-dispersible polymer can include particles having a weight average molecular weight (Mw) of 5,000 to 500,000. In one example, the water-dispersible polymer can range from 50,000 Mw to 300,000 Mw. In some examples, the average particle diameter can be from 10 nm to 5 µm and, as other examples. The particle size distribution of the water-dispersible polymer is not particularly limited, and either polymer having a broad particle size distribution or latex having a mono-dispersed particle size distribution may be used. It is also possible to use two or more kinds of polymer fine particles each having a mono-dispersed particle size distribution in combination.

The water-soluble polymer can be a macromolecule having hydrophilic functional groups, such as -OH, -COOH, -COC. Examples of the water-soluble polymers include, but are not limited to, polyvinyl alcohol, starch derivatives, gelatin, cellulose and cellulose derivatives, polyethylene oxide, polyvinyl pyrrolidone, or acrylamide polymers. By "water-soluble," it is noted that the polymer can be at least partially water-soluble, mostly water-soluble (at least 50%), or in some examples, completely water-soluble (at least 99%).

Water-soluble binders can include starch derivatives such as oxidized starch, etherified starch, and phosphate starch; cellulose derivatives such as methylcellulose, carboxymethylcellulose, and hydroxyethyl cellulose; polyvinyl alcohol derivatives such as polyvinyl alcohol or silanol modified polyvinyl alcohol; natural polymeric resins such as casein, and gelatin or their modified products, soybean protein, pullulan, gum arabic, karaya gum, and albumin or their derivatives; vinyl polymers such as sodium polyacrylate, polyacrylamide, and polyvinylpyrrolidone; sodium alginate; polypropylene glycol; polyethylene glycol; maleic anhydride; or copolymers thereof. In some examples, the binder of the base coating layer can include polyvinyl alcohol and a latex having a glass transition temperature from -50 °C to 35 °C. In one example, the binder of the base coating layer can include a styrene-butadiene copolymer, such Litex^{®} PX 9740 (Synthomer) and a polyvinyl alcohol, such as Mowiol^{®} 4-98 (Kuraray America Inc.).

In some examples, the polymeric binder comprises a water-soluble binder that is a polyvinyl alcohol, a starch derivative, gelatin, a cellulose derivative, a copolymer of vinylpyrrolidone or an acrylamide polymer. In some examples, the polymeric binder comprises a water-dispersible binder that is polyurethane polymer, acrylic polymer or copolymer, vinyl acetate latex, polyester, vinylidene chloride latex, styrene-butadiene or acrylonitrile-butadiene copolymer.

In some examples, the ink-receiving layer might also further comprise, as an optional ingredient, an ink colorant fixing agent or fixative agent. It is believed that the fixing agent can chemically, physically, and/or electrostatically bind a marking material, such as an inkjet ink, at or near an outer surface of the coated print media to provide acceptable water-fastness, smearfastness, and overall image stability. A function of the fixative agent can be thus to reduce ink dry time. In some other examples, the primary layer might also further comprise, as an optional ingredient, a fixative agent. When present, said fixative agent can be similar or different from the fixative agent that could be used in the ink-receiving layer.

The fixative agents can be a metallic salt, a cationic amine polymer, a quaternary ammonium salt, or a quaternary phosphonium salt. The metallic salt may be a water-soluble mono- or a multi-valent metallic salt. The water-soluble metallic salt can be an organic salt or an inorganic salt. The fixative agent can be an inorganic salt. In some examples, the fixative agent is a water-soluble and multi-valent charged salts. Multi-valent charged salts include cations, such as Group I metals, Group II metals, Group III metals, or transition metals, such as sodium, calcium, copper, nickel, magnesium, zinc, barium, iron, aluminum and chromium ions. The associated complex ion can be chloride, iodide, bromide, nitrate, sulfate, sulfite, phosphate, chlorate, acetate ions. The fixative agent can be an organic salt; in some examples, the fixative agent is a water-soluble organic salt; in yet some other examples, the fixative agent is a water-soluble organic acid salt. Organic salt refers to associated complex ion that is an organic specifies, where cations may or may not the same as inorganic salt like metallic cations. Organic metallic salt are ionic compounds composed of cations and anions with a formula such as (CnH2n+1COO-M+)*(H2O)m where M+ is cation species including Group I metals, Group II metals, Group III metals and transition metals such as, for example, sodium, potassium, calcium, copper, nickel, zinc, magnesium, barium, iron, aluminum and chromium ions. Anion species can include any negatively charged carbon species with a value of n from 1 to 35. The hydrates (H₂O) are water molecules attached to salt molecules with a value of m from 0 to 20. Examples of water-soluble organic acid salts include metallic acetate, metallic propionate, metallic formate, metallic oxalate, and the like. The organic salt may include a water-dispersible organic acid salt. Examples of water-dispersible organic acid salts include a metallic citrate, metallic oleate, metallic oxalate, and the like.

In some examples, the fixative agent is a water-soluble, divalent or multi-valent metal salt. Specific examples of the divalent or multi-valent metal salt used in the coating include, but are not limited to, calcium chloride, calcium acetate, calcium nitrate, calcium pantothenate, magnesium chloride, magnesium acetate, magnesium nitrate, magnesium sulfate, barium chloride, barium nitrate, zinc chloride, zinc nitrate, aluminum chloride, aluminum hydroxychloride, and aluminum nitrate. Divalent or multi-valent metal salt might also include CaCl₂, MgCl₂, MgSO₄, Ca(NO₃)₂, and Mg(NO₃)₂, including hydrated versions of these salts. In some examples, the water-soluble divalent or multi-valent salt can be selected from the group consisting of calcium acetate, calcium acetate hydrate, calcium acetate monohydrate, magnesium acetate, magnesium acetate tetrahydrate, calcium propionate, calcium propionate hydrate, calcium gluconate monohydrate, calcium formate and combinations thereof. In some examples, the fixative agent is calcium chloride and/or calcium acetate. In some other examples, the fixative agent is calcium chloride (CaCl₂).

The fixative agent can be present in the ink-receiving layer in an amount representing from about 0.5 wt % to about 20 wt % or in an amount representing from about 1 wt % about 20 wt % of the total dry weight of the ink-receiving layer, for example. In some examples, the ink-receiving layer (120) can include a fixative agent and a binder system wherein the ratio of fixative agent to binder system is from about 1:5 to about. 1:30. In some other examples, the coating layer includes a fixative agent and a binder system wherein the ratio of fixative agent to binder system is from about 1:6 to about1: 15.

In some examples, the ink-receiving layer might also further comprise a COF (coefficient of friction) controlling agent as an optional ingredient. The addition of the COF controlling agent in the image-receiving layer may advantageously assist in maintaining the appropriate COF (coefficient of friction ) of the surface of image-receiving layer in the desired range. The Coefficient of Friction (COF) can be evaluated using the TMI slips and friction tester (model #32-90) per the TAPPI T-549 om-01 method. Such COF controlling agent can also be called "slip aid agent".

In some examples, COF controlling agent can be thermoplastic materials in the form of a dispersion or in the form of an emulsion. The thermoplastic material may be a single thermoplastic material or a combination of two or more thermoplastic materials. Whether used alone or in combination, each thermoplastic materials may have a melting temperature ranging from about 40°C to about 250°C. The COF controlling agent, i.e. thermoplastic material, may be natural materials or polyolefin-based materials. In some examples, the thermoplastic material is a non-ionic material, an anionic material, or a cationic material. In some examples, the thermoplastic material is selected from the group consisting of a beeswax, a carnauba wax, a candelilla wax, a montan wax, a Fischer-Tropsch wax, a polyethylene-based wax, a high density polyethylene-based wax, a polybutene-based wax, a paraffin-based wax, a polytetrafluoroethylene-based material, a polyamide-based material, a polypropylene-based wax, and combinations thereof. In some other examples, the thermoplastic material is an anionic polyethylene wax emulsion, a poly-propylene based thermoplastic material, a high-density polyethylene non-ionic wax micro-dispersion or a high melt polyethylene wax dispersion. In yet some other examples, the thermoplastic material is a high-density polyethylene non-ionic wax micro-dispersion. Examples of suitable thermoplastic materials include Michem^{®} and ResistoCoat^{™} products that are available from Michelman, Inc., Cincinnati, Ohio, and Ultralube^{®} products that are available from Keim Additec Surface GmbH, Kirchberg/Hunsrück.

Some specific examples of the polyethylene-based wax include polyethylene (e.g., Michem^{®} Wax 410), an anionic polyethylene wax emulsion (e.g., Michem^{®} Emulsion 52830, Michem^{®} Lube 103DI, and Michem^{®} Lube 190), an anionic polyethylene wax dispersion (e.g., Michem^{®} Guard 7140), a non-ionic polyethylene wax dispersion (e.g., Michem^{®} Guard 25, Michem^{®} Guard 55, Michem^{®} Guard 349, and Michem^{®} Guard 1350) a non-ionic polyethylene wax emulsion (e.g., Michem^{®} Emulsion 72040), or a high melt polyethylene wax dispersion (e.g., Slip-Ayd^{®} SL 300, Elementis Specialties, Inc., Hightstown, NJ). In some other examples, the thermoplastic material(s) may be an anionic paraffin/ethylene acrylic acid wax emulsion (e.g., Michem^{®} Emulsion 34935), a cationic water based emulsion of polyolefin waxes (e.g., Michem^{®} Emulsion 42035A), anionic microcrystalline wax emulsions (e.g., Michem^{®} Lube 124 and Michem^{®} Lube 124H), or a high density polyethylene/copolymer non-ionic wax emulsion (e.g., Ultralube^{®} E-530V).

The ink-receiving layer and/or the primary layer may also include other optional coating additives such as surfactants, rheology modifiers, defoamers, optical brighteners, biocides, pH controlling agents, dyes, and other additives for further enhancing the properties of the coating. The total amount of optional coating additives may be in the range of 0 to 10 wt % based on the total amount of ingredients. Among these additives, rheology modifier or rheology control agent is useful for addressing runnability issues. Suitable rheology control agents include polycarboxylate-based compounds, polycarboxylated-based alkaline swellable emulsions, or their derivatives. The rheology control agent is helpful for building up the viscosity at certain pH, either at low shear or under high shear, or both. In certain embodiments, a rheology control agent is added to maintain a relatively low viscosity under low shear, and to help build up the viscosity under high shear. It is desirable to provide a coating formulation that is not so viscous during the mixing, pumping and storage stages, but possesses an appropriate viscosity under high shear.

The printable recording media (100) of the present disclosure, that can also be called herein printable recording media, is a media that comprises a base substrate (110). The base substrate (110) can also be called bottom supporting substrate or substrate. The word "supporting" also refers to a physical objective of the substrate that is to carry the coatings layer and the image that is going to be printed. In some examples, the base substrate (110) is a cellulose base substrate meaning thus that the substrate is a cellulose paper. Such cellulose base substrate can be a cellulose paper web.

The cellulose base substrate, or cellulose paper web, can be made of any suitable wood or non-wood pulp. Non-limitative examples of suitable pulp compositions include, but are not limited to, mechanical wood pulp, chemically ground pulp, chemi-mechanical pulp, thermomechanical pulp (TMP) and combinations of one or more of the above. In some examples, the cellulose paper web comprises a bleached hardwood chemical kraft pulp. The bleached hardwood chemical kraft pulp has a shorter fiber structure (about 0.3 to about 0.6 mm length) than soft wood pulp. The shorter fiber structure contributes to good formation of the paper product in roll or sheet form, for example.

Moreover, a filler may be incorporated into the pulp, for example, to substantially control physical properties of the paper product in roll or sheet form. Particles of the filler fill in the void spaces of the fiber network and substantially result in a denser, smoother, brighter and opaque sheet than without a filler. The filler may substantially reduce cost also, since filler is generally cheaper than the pulp itself. Examples of fillers that are incorporated into the pulp include, but are not limited to, ground calcium carbonate, precipitated calcium carbonate, titanium dioxide, kaolin clay, silicates, plastic pigment, alumina trihydrate and combinations of any of the above. An amount of the filler in the pulp may include as much as 15 percent (%) by weight, for example. In some examples, the amount of filler in the pulp ranges from about 0% to about 20% of the paper product in roll or sheet form. In another example, the amount of filler ranges from about 5% to about 15% of the paper product in roll or sheet form. In some examples, if the percentage of filler is more than 20% by weight, pulp fiber-to-fiber bonding may be reduced, which subsequently may decrease stiffness and strength of the resulting paper product in roll or sheet form.

Moreover, an internal sizing may be included, for example. Internal sizing may improve internal bond strength of the pulp fibers, and also may control resistance of the paper product in roll or sheet form to wetting, penetration, and absorption of aqueous liquids. Internal sizing processing may be accomplished by adding a sizing agent to a fiber furnish (or source of the pulp fiber) in the wet-end of paper manufacture. Non-limitative examples of suitable internal sizing agents include a rosin-based sizing agent, a wax-based sizing agent, a cellulose-reactive sizing agent and another synthetic sizing agent, and combinations or mixtures thereof. The degree of internal sizing may be characterized by Hercules Sizing Test (HST) value. In some examples, the cellulose-based paper web has an internal sizing with a low HST value ranging from 1 to 50 (i.e., a soft internal sizing). In some examples, the HST value ranges from about 1 to about 10. Excessive internal sizing may affect the print quality on the paper product, for example, it may cause color-to-color bleed of inks printed on the paper product.

The surface sizing composition according to the principles described herein comprises a macromolecular material, either natural or synthetic, in an amount from about 25% to about 75% dry weight; an inorganic metallic salt in an amount from about 3% to about 20% dry weight; and an amount of an inorganic pigment ranging from greater than 15% to about 60% dry weight in an aqueous mixture, such that a total dry weight equals about 100%. The aqueous mixture is a size press (SP)-applied surface sizing composition in online paper manufacture. In particular, the SP surface sizing composition according to the principles described herein has one or more of a lower content of macromolecular material, a lower content of salt and a higher content of inorganic pigment (filler) than a surface sizing of commercially available office printing paper in the marketplace. In some examples, the SP surface sizing composition according to the principles described herein has each of a lower content of macromolecular material, a lower content of salt and a higher content of inorganic pigment (filler) than the commercially available office printing paper.

The macromolecular material is a high molecular weight material, such as a high molecular weight polymeric material, that functions as both a sizing agent and a binder for the SP surface sizing composition. In some examples, the macromolecular material includes one or both of synthetic polymers and natural polymers. In particular, by definition, the macromolecular material one or more of is water-soluble or water-dispersible, has strong film forming capability, and can bind particles of the inorganic pigment to form a coating layer. Moreover, by definition, the macromolecular material is inert to the inorganic metallic salt. The term 'film-forming' as used herein means that, during drying, or i.e., when aqueous solvent is removed from the cellulose-based paper web, the macromolecules can form continuous network, or latex particles can aggregated together to form a continuous film, or a continuous barrier layer to the aqueous solvent or moisture at a macroscopic level. The term 'inert' as used herein means that the macromolecular material will not interact with a fixative so as to cause the polymers to be precipitated, gelled, or form any kind of solid particle, which would adversely reduce a binding capability of the macromolecular material and a coating ability of the SP surface sizing composition.

Examples of a synthetic polymer useful in the macromolecular material include, but are not limited to, polyvinyl alcohol, polyvinyl pyrrolidone, acrylic latex, styrene-butadiene latex, polyvinyl acetate latex, and a copolymer latex of any of the above-named monomers, and combinations or mixtures thereof. Examples of a natural polymer useful in the macromolecular material include, but are not limited to, casein, soy protein, a polysaccharide, a cellulose ether, an alginate, a virgin starch and a modified starch, and a combination of any of the above-named polymers. The starch species includes, but is not limited to, corn starch, potato starch, derivatized starch and modified starch including, but not limited to, ethylated starch, oxidized starch, anionic starch, and cationic starch. For example, an ethylated starch, such as K96F from Grain Processing Corp., Muscatine, IA, or a hydroxyethyl ether derivatized corn starch, such as Penford^{®} 280 Gum (i.e., 2-hydroxyethyl starch ether, hydroxyethyl starch or ethylated starch) from Penford Products Co., Cedar Rapids, IA, may be used.

The printable recording media, described herein, is prepared by using several surface treatment compositions herein named a coating layer or coating composition. A method of making a coated print media includes applying a coating composition as a layer to a media substrate and drying the coating composition to remove water from the media substrate to leave an ink-receiving layer and a primary layer if needed thereon.

In some examples, as illustrated in Figure 5, a method (200) of making a printable recording media encompasses: providing (210) a base substrate (110) with an image-side and a back-side; applying (210) an ink-receiving layer (120) comprising a reactive crosslinking agent, inorganic pigment particles or a mixture of inorganic particles, and polymeric binders or a mixture of polymeric binders to the image-side of the base substrate; and drying (220) the coating composition to remove water from the media substrate to leave an ink-receiving layer thereon in order to obtain the printable media. In some examples, the ink-receiving layer (120) is applied to the base substrate (110) on the image receiving side of the printable media. In some other examples, the ink-receiving layer (120) is applied to the supporting base substrate (110) on the image receiving side (101) and on the backside (102) of the printable media.

The method of making a coated printable recording media encompasses: providing a base substrate (110), with an image-side and a back-side; applying a primary layer (130) comprising, at least, inorganic pigment particles or a mixture of inorganic particles and polymeric binders or a mixture of polymeric binders, on the image-side of the base substrate (110) and then applying an ink-receiving layer (120) comprising a reactive crosslinking agent, inorganic pigment particles or a mixture of inorganic particles, and polymeric binders or a mixture of polymeric binders over the primary layer on the image-side of the base substrate.

The coating layer (120) and the primary layer (130), can be applied to the base substrate (110) by using any method appropriate for the coating application properties, e.g., thickness, viscosity, etc. Non-limiting examples of methods include size press, slot die, blade coating, Meyer rod coating and padding coating. In another example, a two rolls padding coating is used to apply the coating composition to a substrate (or other type of substrate).

In some examples, the coating layers can be applied in one single production run. When the coating layer are present on both sides of the base substrates, depending on set-up of production machine in a mill, both sides of the substrate may be coated during a single manufacture pass, or each side is coated in a separate pass. Subsequently, when the coating composition is dried, it can form an ink-receiving layer. Drying can be by air drying, heated airflow drying, baking, infrared heated drying, etc. Other processing methods and equipment can also be used. For one example, the coated media substrate can be passed between a pair of rollers, as part of a calendering process, after drying. The calendering device can be any kind of calendaring apparatus, including but not limited to off-line super-calender, on-line calender, softnip calender, hard-nip calender, or the like. Once applied to the image-side (101) of the base substrate (110), the ink-receiving layer (120), and the primary layer can be calendered. The calendaring can be done either in room temperature or at an elevated temperature and/or pressure. In one example, the elevated temperature can range from 40°C to 60°C. In one example, the calender pressure can range from about 689 kPa (100 psi) to about 13789 kPa (2,000 psi). The image-receiving coating layer (120) and, when present, the primary layer (130), can be dried using any drying method in the arts such as box hot air dryer. The dryer can be a single unit or could be in a serial of 3 to 7 units so that a temperature profile can be created with initial higher temperature (to remove excessive water) and mild temperature in end units (to ensure completely drying with a final moisture level of less than 1-5 % for example). The peak dryer temperature can be programmed into a profile with higher temperature at begging of the drying when wet moisture is high and reduced to lower temperature when web becoming dry. The dryer temperature is controlled to a temperature of less than about 120°C to avoid reaction on reactive crosslink chemical agent, and the web temperature is controlled in the range of about 80 to about 100°C. In some examples, the operation speed of the coating/drying line is 20 to 30 meters per minute.

Once the coating compositions are applied to the base substrate and appropriately dried, ink compositions can be applied by any processes onto the printable recording media. In some examples, the ink composition is applied to the printable recording media via inkjet printing techniques. A printing method could encompasses obtaining a coated printable media as defined herein and applying an ink composition onto said printable recording media to form a printed image. Said printed image will have, for instance, enhanced image quality and image permanence. In some examples, when needed, the printed image can be dried using any drying device attached to a printer such as, for instance, an IR heater.

The method for producing printed images, or printing method, includes providing a printable recording media such as defined herein; applying an ink composition on the coating layer of the print media, to form a printed image; and drying the printed image in a hot air or IR heated dryer in order to complete crosslink reaction and then provide, for example, a printed image with enhanced quality and enhanced image permanence. In some examples, the printing method for producing images is an inkjet printing method. By inkjet printing method, it is meant herein a method wherein a stream of droplets of ink is jetted onto the recording substrate or media to form the desired printed image. The ink composition may be established on the recording media via any suitable inkjet printing technique. Examples of inkjet method include methods such as a charge control method that uses electrostatic attraction to eject ink, a drop-on-demand method which uses vibration pressure of a Piezo element, an acoustic inkjet method in which an electric signal is transformed into an acoustic beam and a thermal inkjet method that uses pressure caused by bubbles formed by heating ink. Non-limitative examples of such inkjet printing techniques include thus thermal, acoustic and piezoelectric inkjet printing. In some examples, the ink composition is applied onto the recording media using inkjet nozzles. In some other examples, the ink composition is applied onto the recording method using thermal inkjet printheads.

In some examples, the printing method is a capable of printing more than about 15.2 meter per minute (50 feet per minute (fpm)) (i.e. has a print speed that is more than about 50 fpm). The printing method described herein can be thus considered as a high-speed printing method. The web-speed could be from about 30.5 to 1219.2 meter/min (100 to about 4 000 feet per minute (fpm)). In some other examples, the printing method is a printing method capable of printing from about 30.5 to 304.8 meter/min (100 to about 1 000 feet per minute). In yet some other examples, the printing method is capable of printing at a web-speed of more than about 61.0 meter/min (200 feet per minute (fpm)). In some example, the printing method is a high-speed web press printing method. As "web press", it is meant herein that the printing technology encompasses an array of inkjet nozzles that span the width of the paper web. The array is thus able, for example, to print on 20", 30", and 42" wide web or on rolled papers.

In some examples, the printing method as described herein prints on one-pass only. The paper passes under each nozzle and printhead only one time as opposed to scanning type printers where the printheads move over the same area of paper multiple times and only a fraction of total ink is used during each pass. The one-pass printing puts 100% of the ink from each nozzle/printhead down at once and is therefore more demanding on the ability of the paper to handle the ink in a very short amount of time.

As mentioned above, a print media in accordance with the principles described herein may be employed to print images on one or more surfaces of the print media. In some examples, the method of printing an image includes depositing ink that contains particulate colorants. A temperature of the print media during the printing process is dependent on one or more of the nature of the printer, for example. Any suitable printer may be employed such as, but not limited to, offset printers and inkjet printers. In some examples, the printer is a HP T350 Color Inkjet Webpress printer (Hewlett Packard Inc.). The printed image may be dried after printing. The drying stage may be conducted, by way of illustration and not limitation, by hot air, electrical heater or light irradiation (e.g., IR lamps), or a combination of such drying methods. In order to achieve best performances, it is advisable to dry the ink at a maximum temperature allowable by the print media that enables good image quality without deformation. Examples of a temperature during drying are, for examples, from about 100°C to about 205°C, or from about 120°C to about 180°C. The printing method may further include a drying process in which the solvent (such as water), that can be present in the ink composition, is removed by drying. As a further step, the printable recording media can be submitted to a hot air-drying systems. The printing method can also encompass the use of a fixing agent that will retain with the pigment, present in the ink composition that has been jetted onto the media.

In some examples, the ink composition is an inkjet ink composition that contains one or more colorants that impart the desired color to the printed message and a liquid vehicle. As used herein, "colorant" includes dyes, pigments, and/or other particulates that may be suspended or dissolved in an ink vehicle. The colorant can be present in the ink composition in an amount required to produce the desired contrast and readability. In some examples, the ink compositions include pigments as colorants. Pigments that can be used include self-dispersed pigments and non-self-dispersed pigments. Any pigment can be used; suitable pigments include black pigments, white pigments, cyan pigments, magenta pigments, yellow pigments, or the like. Pigments can be organic or inorganic particles as well known in the art. As used herein, "liquid vehicle" is defined to include any liquid composition that is used to carry colorants, including pigments, to a substrate. A wide variety of liquid vehicle components may be used and include, as examples, water or any kind of solvents.

Reference throughout the specification to "one example", "another example", "an example", and so forth, means that a particular element (e.g., feature, structure, and/or characteristic) described in connection with the example is included in at least one example described herein, and may or may not be present in other examples. In addition, it is to be understood that the described elements for any example may be combined in any suitable manner in the various examples unless the context clearly dictates otherwise. In describing and claiming the examples disclosed herein, the singular forms "a", "an", and "the" include plural referents unless the context clearly dictates otherwise.

As used herein, the term "about" is used to provide flexibility to a numerical range endpoint by providing that a given value may be "a little above" or "a little below" the endpoint. The degree of flexibility of this term can be dictated by the particular variable and would be within the knowledge of those skilled in the art to determine based on experience and the associated description herein.

The term "acid value" or "acid number" refers to the mass of potassium hydroxide (KOH) in milligrams that can be used to neutralize one gram of substance (mg KOH/g), such as the latex polymers disclosed herein. This value can be determined, in one example, by dissolving or dispersing a known quantity of a material in organic solvent and then titrating with a solution of potassium hydroxide (KOH) of known concentration for measurement.

The term "(meth)acrylate," "(meth)acrylic," or "(meth)acrylic acid," or the like refers to monomers, copolymerized monomers, etc., that can either be acrylate or methacrylate (or a combination of both), or acrylic acid or methacrylic acid (or a combination of both). This can be the case for either dispersant polymer for a pigment dispersion or for dispersed polymer binder particles that may include co-polymerized acrylate and/or methacrylate monomers. Also, in some examples, the terms "(meth)acrylate" and "(meth)acrylic" can be used interchangeably, as acrylates and methacrylates described herein include salts of acrylic acid and methacrylic acid, respectively. Thus, mention of one compound over another can be a function of pH. Furthermore, even if the monomer used to form the polymer was in the form of a (meth)acrylic acid during preparation, pH modifications during preparation or subsequently when added to an ink composition can impact the nature of the moiety as well (acid form vs. salt form). Thus, a monomer or a moiety of a polymer described as (meth)acrylic acid or as (meth)acrylate should not be read so rigidly as to not consider relative pH levels, and other general organic chemistry concepts.

As used herein, "liquid vehicle" or "ink vehicle" refers to a liquid fluid in which colorant, such as pigments, can be dispersed and otherwise placed to form an ink composition. A wide variety of liquid vehicles may be used with the systems and methods of the present disclosure. Such liquid vehicles may include a mixture of a variety of different agents, including, water, organic co-solvents, surfactants, anti-kogation agents, buffers, biocides, sequestering agents, viscosity modifiers, surface- active agents, water, etc.

As used herein, "pigment" generally includes pigment colorants.

As used herein, a plurality of items, structural elements, compositional elements, and/or materials may be presented in a common list for convenience. However, these lists should be construed as though each member of the list is individually identified as a separate and unique member. Thus, no individual member of such list should be construed as a de facto equivalent of any other member of the same list solely based on their presentation in a common group without indications to the contrary.

Concentrations, dimensions, amounts, and other numerical data may be presented herein in a range format. It is to be understood that such range format is used merely for convenience and brevity and should be interpreted flexibly to include not only the numerical values explicitly recited as the limits of the range, but also to include all the individual numerical values or sub-ranges encompassed within that range as if each numerical value and sub-range is explicitly recited. For example, a weight ratio range of about 1 wt % to about 20 wt % should be interpreted to include not only the explicitly recited limits of about 1 wt % and about 20 wt % , but also to include individual weights such as 2 wt % , 11 wt % , 14 wt % , and sub-ranges such as 10 wt % to 20 wt % , 5 wt % to 15 wt % , etc. In some other examples, a range of 1 part to 20 parts should be interpreted to include not only the explicitly recited concentration limits of about 1 part to about 20 parts, but also to include individual concentrations such as 2 parts, 3 parts, 4 parts, etc. All parts are dry parts in unit weight, with the sum of all the coating components equal to 100 parts, unless otherwise indicated.

To further illustrate the present disclosure, an example is given herein. It is to be understood this example is provided for illustrative purposes and is not to be construed as limiting the scope of the present disclosure.

### EXAMPLES

The raw materials and chemical components used in the illustrating samples are listed in Table 1.

**Table 1**

| **Ingredients** | **Nature of the ingredients** | **Supplier** |
|---|---|---|
| Disponil^{®}AFX 4030 | Surfactant | BASF Co |
| Covercarb^{®} 85 | Particulate filler | Omya Co |
| Opercarb^{®} A 40 | Particulate filler | Specialty Minerals |
| Novajet^{®} 3800 | Polymeric binder | Omnova Solutions |
| Mowiol^{®} 13-88 | Polymeric binder | Clariant |
| CaCl2 | Colorant fixing agent | Aldrich |
| Sodium Hydroxide | pH control agent | Aldrich |
| Fulacolor^{®} | Particulate filler | BYK |
| Albacar^{®} HO | Particulate filler | Specialty Minerals |
| Rovene^{®} 6023 | Polymeric binder | Creek Polymers |
| Polycup^{®} 7360A | Crosslinker | Solenis Inc |
| EC-1722 | COF control | Faci Co |
| Acetate acid/NaOH | pH control agent | Aldrick |

### Example 1 - Preparation of printable recording media samples

Different media were made using different coating compositions (Primary coating composition and Image receiving coating composition). Such compositions are prepared by mixing the ingredients, in water, as illustrated in table 2 and 3. Chemicals are mixed together in a tank by using normal stirring equipment. Each coating layer compositions is applied on the on the image side of a raw base substrate (110) at a coat-weight of about 10 gram/square meter (gsm) using a Meyer rod in lab in view of obtaining media samples I to V. The base supporting paper substrate used is 45# book paper from Evergreen^{®}. The recording media are then calendered through a lab soft nip calendar machine (at13789 kPa (2000 psi) at room temperature). The formulations of the ink-receiving layer (130) and of the primary coating layer (120) are illustrated, respectively, in the Tables 2, and 3 below. Each number represent the dry parts number of each ingredient in the dry composition.

**Table 2**

| **primary coating layer (130)** | | |
|---|---|---|
| **Chemical Components** | **Exp-P-A** | **Exp-P-B** |
| Disponil^{®} AFX 4030 | 0.3 | 0.3 |
| Covercarb^{®} 85 | 100.0 | 70.0 |
| Opercarb^{®} A 40 | - | 30.0 |
| Novajet^{®} 3800 | 10.0 | 10.0 |
| Mowiol^{®} 13-88 | 2.0 | 2.0 |
| CaCl2 | 5.0 | 5.0 |
| Sodium Hydroxide | 0.1 | 0.1 |

**Table 3**

| **Image receiving coating (120)** | | | |
|---|---|---|---|
| **Chemical Components** | **Exp-IR-A** | **Exp-IR-B** | **Exp-IR-C** |
| Fulacolor^{®} | 100.0 | 80.0 | 100.0 |
| Albacar^{®} HO | - | 20.0 | - |
| Rovene^{®} 6023 | 10.0 | 10.0 | 10.0 |
| Mowiol^{®} 13-88 | 2.0 | 2.0 | 2.0 |
| Polycup^{®} 7360A | 5.0 | 5.0 | - |
| CaCl2 | 1.5 | 1.5 | 1.5 |
| EC-1722 | 3.0 | 3.0 | 3.0 |
| Acetate acid/NaOH | adjust pH to 5.5-6.5 | adjust pH to 5.5-6.5 | adjust pH to 5.5-6.5 |

Different media (samples 1 to 3) are made using the different coating formulations. The media sample structures are illustrated in Table 4.

**Table 4**

| **Media** | **primary coating layer (130)** | **Image receiving coating (120)** |
|---|---|---|
| Sample 1 | Exp-P-A | Exp-IR-A |
| Sample 2 | Exp-P-B | Exp-IR-B |
| Sample 3 | Exp-P-A | Exp-IR-C |

### Example 2 - Samples performances

The same images are printed on the media samples 1, 2 and 3 . The samples are printed using an HP CM8060 MFP printer with web press inkjet inks in the pens. The prints were made in 2 pass/ 6 dry spin mode. The resulting printed medias are evaluated for different performances: printing quality, gloss, durability (Scratch resistances, ink abrasions). The results of these tests are expressed in the Table 5 below.

Image quality is evaluated using both numeric measurement method and visual evaluation method. The KOD and COD (Black and Cyan optical density) is evaluated using a X-Rite Spectro-densitometer. The color gloss was measured using a BYK Gardner Gloss Meter at 75 degrees. A higher score means a better performance. The color gloss of black and cyan were measured and the minimum color gloss was reported. Bleed and Coalescence (both related to image quality) was checked by printing a black line on a solid yellow color square to see how much ink spread from black line into yellow color. A black line was also printed on a solid blue solid color square to determine the uniformity of the solid blue square after printing the black line thereon. Image quality ratings were based on the following scores: 5-No bleed and no coalescence; 4-Very slight bleed and coalescence; 3-Moderate bleed and coalescence; 2-Significant bleed and coalescence; and 1- Ink flow.

Resistance tests are performed onto the obtained printed media. The printed media sample are tested for durability immediately after printing. The resistance test refers to the ability of a printed image to resist appearance degradation upon rubbing the image. Good resistance, upon rubbing, will tend to not transfer ink from a printed image to surrounding areas where the ink has not been printed.

The eraser durability test was performed by mounting a pencil eraser on a force spring to provide a consistent force of 2.25 kg force over a 3.2 cm² (0.5 square inch) eraser area. The eraser was then pressed against the print and drawn down. The durability was rated according to the following scale. 5: no damage; 4: very slight damage; 3: some ink gone; 2: more than half of ink removed; 1: white paper is visible, total ink damage or transfer.

Wet rub durability was checked visually. Seven strips of color (black, blue, red, green, cyan, magenta, and yellow) were printed at the top of a coated sample. A cloth square was attached to the Taber Linear Abraser tip and wet with deionized water. The cloth covered tip was then placed onto the printed image and moved through each printed line in one motion (25 cycles/min) before being lifted off the sheet. Damage ratings were based on the following scores: 5-No damage; 4-Some ink transfer to cloth; 3-Moderate ink removal and transfer to cloth; 2-Significant ink removal and transfer to cloth; and 1-Full ink removal.

The resulting printed articles are also tested with a Sutherland^{®} Ink Rub tester with 0.91 kg (2lb) weigh and 5 cycles (in accordance with ASTM D-5264). It is designed to evaluate the scuffing or rubbing resistance of the printed or coated surface of paper, paperboard, film and other materials. The Sutherland^{®} Ink Rub tester features a digital counter with a fiber optic sensor for accuracy and is compatible with the requirements of the ASTM D-5264 test method. on normal and heated condition). The "visual difference" in the printed surface are visually rated (with a score between 1 and 5, 1 is worst, 5 is best).

It can be seen that the examples with the recording media sample with the coating that ink-receiving layer, comprising the reactive crosslinking agent, (Sample 1 and 2) can have increased gloss, durability and image quality.

**Table 5**

| **Test items** | **Results** | | |
|---|---|---|---|
| | **Sample 1** | **Sample 2** | **Sample 3 (comparative)** |
| Sheet gloss (75 degree) | 74 | 67 | 75 |
| K- gloss | 86 | 78 | 85 |
| C- gloss | 83 | 72 | 82 |
| COD | 1.38 | 1.26 | 1.41 |
| KOD | 1.46 | 1.38 | 1.47 |
| Max Coalescence | 2.57 | 2.2 | 2.16 |
| K/Y Bleed | 5 | 5 | 5 |
| Hot roller test | 5 | 5 | 2 |
| Sutherland scratch test | 4+ | 5 | 2.5 |
| Wet Taber test | 5 | 5 | 1 |
| Eraser test immediate after printing | 5 | 5 | 3 |

## Claims

1. A printable recording media comprising:
a. a base substrate with an image-side and a back-side;
b. and an ink-receiving layer, applied to the image-side of the base substrate, comprising, at least, a reactive crosslinking agent, inorganic pigment particles or a mixture of inorganic particles, and polymeric binders or a mixture of polymeric binders; and **characterized in that** the printable recording media comprises:
c. a primary layer containing, at least, inorganic pigment particles or a mixture of inorganic particles, and polymeric binders or a mixture of polymeric binders, that is applied on the image-side of the base substrate, below the ink-receiving layer;
and wherein the reactive crosslinking agent is an azetidinium-containing polyamine polymer.

2. The printable recording media of claim 1 wherein the ink-receiving layer has a coat-weigh ranging from about 0.5 gsm to about 20 gsm.

3. The printable recording media of claim 1 wherein the primary layer has a coat-weigh ranging from about 3 gsm to about 50 gsm.

4. The printable recording media according to claim 1 wherein the ink-receiving layer is applied is applied to both opposing sides of the base substrate.

5. The printable recording media according to claim 1 wherein the reactive crosslinking agent is present in the ink-receiving layer in an amount representing from about 0.5 wt % to about 15 wt % of the total weight of the ink-receiving coating composition.

6. The printable recording media according to claim 1 wherein the reactive crosslinking agent includes the structure: where R₁ is a substituted or unsubstituted C₂-C₁₂ linear alkylene group and R₂ is H or CH₃.

7. The printable recording media of claim 1 wherein the ink-receiving layer further includes fixative agents.

8. The printable recording media of claim 7 wherein the fixative agent is a metallic salt, a cationic amine polymer, a quaternary ammonium salt, or a quaternary phosphonium salt.

9. The printable recording media of claim 1 wherein, in the ink-receiving layer, the polymeric binder and/or mixture of polymeric binders are present in an amount representing from about 1 wt % to about 18 wt % with respect to the total dry weight of the ink-receiving layer.

10. A method for forming a printable recording media comprising:
a. providing a base substrate, with an image-side and a back-side;
b. applying an ink-receiving layer comprising a reactive crosslinking agent, inorganic pigment particles or a mixture of inorganic particles, and polymeric binders or a mixture of polymeric binders to the image-side of the base substrate; wherein the reactive crosslinking agent is an azetidinium-containing polyamine polymer;
c. wherein a primary layer comprising, at least, inorganic pigment particles or a mixture inorganic particles and polymeric binders or a mixture of polymeric binders, is applied on the image-side of the base substrate below the ink-receiving layer;
d. and drying the ink-receiving layer to remove water from the media substrate to leave an ink-receiving layer thereon.

11. A printing method comprising:
a. obtaining a printable recording media comprising a base substrate with an image-side and a back-side, and an ink-receiving layer, applied to the image-side of the base substrate, comprising a reactive crosslinking agent, inorganic pigment particles or a mixture of inorganic particles, and polymeric binders or a mixture of polymeric binders; and a primary layer containing, at least, inorganic pigment particles or a mixture of inorganic particles, and polymeric binders or a mixture of polymeric binders, that is applied on the image-side of the base substrate, below the ink-receiving layer;
and wherein the reactive crosslinking agent is an azetidinium-containing polyamine polymer;
b. and applying an ink composition onto said printable recording media to form a printed image.

## Patentansprüche

1. Bedruckbares Aufzeichnungsmedium, das Folgendes umfasst:
a. ein Basissubstrat mit einer Bildseite und einer Rückseite;
b. und eine auf die Bildseite des Basissubstrats aufgebrachte Tintenaufnahmeschicht, die mindestens ein reaktives Vernetzungsmittel, anorganische Pigmentpartikel oder eine Mischung anorganischer Partikel, und polymere Bindemittel oder eine Mischung polymerer Bindemittel umfasst; **dadurch gekennzeichnet, dass** das druckbare Aufzeichnungsmedium Folgendes umfasst:
c. eine Primärschicht, die mindestens anorganische Pigmentpartikel oder eine Mischung anorganischer Partikel, und polymere Bindemittel oder eine Mischung polymerer Bindemittel enthält, die auf der Bildseite des Basissubstrats unter der Tintenaufnahmeschicht aufgebracht ist;
und wobei das reaktive Vernetzungsmittel ein azetidiniumhaltiges Polyaminpolymer ist.

2. Bedruckbares Aufzeichnungsmedium nach Anspruch 1, wobei die Tintenaufnahmeschicht ein Beschichtungsgewicht, das von 0,5 g/m² bis etwa 20 g/m² reicht, aufweist.

3. Bedruckbares Aufzeichnungsmedium nach Anspruch 1, wobei die Primärschicht ein Beschichtungsgewicht in einem Bereich von etwa 3 g/m² bis etwa 50 g/m² aufweist.

4. Bedruckbares Aufzeichnungsmedium nach Anspruch 1, wobei die Tintenaufnahmeschicht auf beiden gegenüberliegenden Seiten des Basissubstrats aufgebracht ist.

5. Bedruckbares Aufzeichnungsmedium nach Anspruch 1, wobei das reaktive Vernetzungsmittel in der Tintenaufnahmeschicht in einer Menge vorhanden ist, die etwa 0,5 Gewichtsprozent bis etwa 15 Gewichtsprozent des Gesamtgewichts der Tintenaufnahmebeschichtungszusammensetzung entspricht.

6. Bedruckbares Aufzeichnungsmedium nach Anspruch 1, wobei das reaktive Vernetzungsmittel die Folgende Struktur einschließt: wobei R₁ eine substituierte oder unsubstituierte lineare C₂ -C₁₂-Alkylengruppe und R₂ H oder CH₃ ist.

7. Bedruckbares Aufzeichnungsmedium nach Anspruch 1, wobei die Tintenaufnahmeschicht ferner Fixiermittel einschließt.

8. Bedruckbares Aufzeichnungsmedium nach Anspruch 7, wobei das Fixiermittel ein Metallsalz, ein kationisches Aminpolymer, ein quaternäres Ammoniumsalz oder ein quaternäres Phosphoniumsalz ist.

9. Bedruckbares Aufzeichnungsmedium nach Anspruch 1, wobei in der Tintenaufnahmeschicht das Polymerbindemittel und/oder die Mischung aus Polymerbindemitteln in einer Menge vorhanden sind, die etwa 1 Gewichtsprozent bis etwa 18 Gewichtsprozent, bezogen auf das Gesamttrockengewicht der Tintenaufnahmeschicht, entspricht.

10. Verfahren zum Bilden eines bedruckbaren Aufzeichnungsmediums, das Folgendes umfasst:
a. Bereitstellen eines Basissubstrats mit einer Bildseite und einer Rückseite;
b. Aufbringen einer Tintenaufnahmeschicht, die ein reaktives Vernetzungsmittel, anorganische Pigmentpartikel oder eine Mischung anorganischer Partikel, und polymere Bindemittel oder eine Mischung polymerer Bindemittel umfasst, auf die Bildseite des Basissubstrats; wobei das reaktive Vernetzungsmittel ein azetidiniumhaltiges Polyaminpolymer ist;
c. wobei eine Primärschicht, die mindestens anorganische Pigmentpartikel oder eine Mischung anorganischer Partikel, und polymere Bindemittel oder eine Mischung polymerer Bindemittel umfasst, auf der Bildseite des Basissubstrats unter der Tintenaufnahmeschicht aufgebracht ist;
d. und Trocknen der Tintenaufnahmeschicht, um Wasser von dem Mediensubstrat zu entfernen und eine Tintenaufnahmeschicht darauf zurückzulassen.

11. Druckverfahren, das Folgendes umfasst:
a. Erhalten eines bedruckbaren Aufzeichnungsmediums, das ein Basissubstrat mit einer Bildseite und einer Rückseite, und eine auf die Bildseite des Basissubstrats aufgebrachte Tintenaufnahmeschicht, die mindestens ein reaktives Vernetzungsmittel, anorganische Pigmentpartikel oder eine Mischung anorganischer Partikel, und polymere Bindemittel oder eine Mischung polymerer Bindemittel umfasst, umfasst; und eine Primärschicht, die mindestens anorganische Pigmentpartikel oder eine Mischung anorganischer Partikel, und polymere Bindemittel oder eine Mischung polymerer Bindemittel enthält, die auf der Bildseite des Basissubstrats unter der Tintenaufnahmeschicht aufgebracht ist;
und wobei das reaktive Vernetzungsmittel ein azetidiniumhaltiges Polyaminpolymer ist;
b. und Aufbringen einer Tintenzusammensetzung auf das bedruckbare Aufzeichnungsmedium, um ein gedrucktes Bild zu bilden.

## Revendications

1. Support d'enregistrement imprimable comprenant :
a. un substrat de base avec un côté image et un côté arrière ;
b. et une couche de réception d'encre, appliquée sur le côté image du substrat de base, comprenant, au moins, un agent de réticulation réactif, des particules de pigment inorganiques ou un mélange de particules inorganiques, et des liants polymères ou un mélange de liants polymères ; et
**caractérisé en ce que** le support d'enregistrement imprimable comprend :
c. une couche primaire contenant, au moins, des particules de pigment inorganiques ou un mélange de particules inorganiques, et des liants polymères ou un mélange de liants polymères, qui est appliquée sur le côté image du substrat de base, sous la couche de réception d'encre ;
et dans lequel l'agent de réticulation réactif est un polymère de polyamine contenant de l'azétidinium.

2. Support d'enregistrement imprimable selon la revendication 1, dans lequel la couche de réception d'encre a un poids de revêtement se situant dans une plage allant d'environ 0,5 gsm à environ 20 gsm.

3. Support d'enregistrement imprimable selon la revendication 1, dans lequel la couche primaire a un poids de revêtement se situant dans une plage allant d'environ 3 gsm à environ 50 gsm.

4. Support d'enregistrement imprimable selon la revendication 1, dans lequel la couche de réception d'encre est appliquée sur les deux côtés opposés du substrat de base.

5. Support d'enregistrement imprimable selon la revendication 1, dans lequel l'agent de réticulation réactif est présent dans la couche de réception d'encre dans une quantité représentant d'environ 0,5 % en poids à environ 15 % en poids du poids total de la composition de revêtement de réception d'encre.

6. Support d'enregistrement imprimable selon la revendication 1, dans lequel l'agent de réticulation réactif comprend la structure : où R₁ représente un groupe alkylène linéaire C₂-C₁₂ substitué ou non substitué et R₂ représente H ou CH₃.

7. Support d'enregistrement imprimable selon la revendication 1, dans lequel la couche de réception d'encre comporte en outre des agents fixateurs.

8. Support d'enregistrement imprimable selon la revendication 7, dans lequel l'agent fixateur est un sel métallique, un polymère aminé cationique, un sel d'ammonium quaternaire ou un sel de phosphonium quaternaire.

9. Support d'enregistrement imprimable selon la revendication 1 dans lequel, dans la couche de réception d'encre, le liant polymère et/ou le mélange de liants polymères sont présents en une quantité représentant d'environ 1 % en poids à environ 18 % en poids par rapport au poids sec total de la couche de réception d'encre.

10. Procédé de formation d'un support d'enregistrement imprimable comprenant :
a. la fourniture d'un substrat de base, avec un côté image et un côté arrière ;
b. l'application d'une couche de réception d'encre comprenant un agent de réticulation réactif, des particules de pigment inorganiques ou un mélange de particules inorganiques, et des liants polymères ou un mélange de liants polymères sur le côté image du substrat de base ; dans lequel l'agent de réticulation réactif est un polymère de polyamine contenant de l'azétidinium ;
c. dans lequel une couche primaire comprenant, au moins, des particules de pigment inorganiques ou un mélange de particules inorganiques et des liants polymères ou un mélange de liants polymères, est appliquée sur le côté image du substrat de base sous la couche de réception d'encre ;
d. et le séchage de la couche de réception d'encre pour éliminer de l'eau du substrat du support afin de laisser une couche de réception d'encre sur celui-ci.

11. Procédé d'impression comprenant :
a. l'obtention d'un support d'enregistrement imprimable comprenant un substrat de base avec un côté image et un côté arrière, et une couche de réception d'encre, appliquée sur le côté image du substrat de base, comprenant un agent de réticulation réactif, des particules de pigment inorganiques ou un mélange de particules inorganiques, et des liants polymères ou un mélange de liants polymères ; et une couche primaire contenant, au moins, des particules de pigment inorganiques ou un mélange de particules inorganiques, et des liants polymères ou un mélange de liants polymères, qui est appliquée sur le côté image du substrat de base, sous la couche de réception d'encre ;
et dans lequel l'agent de réticulation réactif est un polymère de polyamine contenant de l'azétidinium ;
b. et l'application d'une composition d'encre sur ledit support d'enregistrement imprimable pour former une image imprimée.
